

## UNITED STATES PATENT OFFICE.

ALBERT CHEVALIER, OF PARIS, FRANCE, ASSIGNOR TO SOCIETE DU FEUTRE, OF PARIS, FRANCE.

## METHOD FOR CARROTTING FUR AND HAIR.

No Drawing.

Application filed February 2, 1921. Serial No. 441,851.

To all whom it may concern:

Be it known that I, ALBERT CHEVALIER, citizen of the French Republic, residing at Paris, Seine, in the Republic of France, have 5 invented new and useful Improvements in Methods for Carrotting Fur and Hair, of which the following is a specification.

The operation known as carrotting consists in dissolving or attacking by suitable 10 means the cuticle of the hair to be used in the manufacture of felt in such manner as to release the end of the series of scales whose assemblage constitutes the surface of the hair.

15 My invention consists in an improved method for carrotting hair, for use in the manufacture of hats in which method alkali-metal or alkaline earth sulphides are employed in pure water or in a slightly alkaline 20 solution.

The alkali-metal and alkaline earth sulphides have the property of dissolving the 25 productions of the epidermis such as hair, feathers or horn with more or less efficacy according to the particular sulphide employed. Concentrated solutions of these sulphides will entirely dissolve the hair, but their action may be regulated by suitably diluting the same whereby only the surface portion 30 of the hair shall be attacked and the sulphide shall be unable to continue its action by reason of the rapid oxidation thereof upon contact with the air.

35 The advantages obtained by the use of sulphides for the carrotting operation are considerable.

The ripening process for the hair may be dispensed with. The hair which is prepared by my process is of such nature as to be 40 felted immediately after the carrotting is effected and without being obliged to wait for several months for the ripening of the hair as in the known methods. The felt which is thus obtained will possess all the 45 necessary properties as regards tenacity and fineness of grain.

Tanning of the skins after the carrotting

process is rendered possible. In the known methods it is impossible to make use of the skins after the removal of the hair except 50 in the shape of raw material for glue manufacture. The skins are in fact attacked more or less by the acid liquids or vapors used, and the high temperature of the drying room causes the skin to lose its normal 55 strength.

In the process according to my invention, the skins are not attacked nor is a high temperature employed, and for this reason the skins may be treated by the current methods 60 of hair removal in view of the subsequent tanning of the same.

By way of example, in accordance with my improved method, the skins are brushed over with a 4 per cent solution of monosulphide of sodium in pure or slightly alkaline 65 water. The skins are dried either in the open air or in a drying room provided with a considerable supply of air. They are ready for use immediately after the drying 70 operation is completed.

Having now described my invention, what I claim as new and desire to secure by Letters Patent is:

1. A process for carrotting hair for use in 75 the manufacture of hats, which process consists in subjecting animal skins to the action of a soluble metallic sulphide and allowing the skins to dry in the presence of air, thereby causing oxidation of the sulphide solution and checking the destructive action of 80 said solution.

2. A process for carrotting hair for use in the manufacture of hats, which process consists in brushing animal skins with a 4% 85 solution of monosulphide of sodium and allowing the skins to dry rapidly in the presence of air and cause oxidation of said solution and also check the destructive action of 90 said solution.

In testimony whereof I have signed my name to this specification.

ALBERT CHEVALIER.